

## UNITED STATES PATENT OFFICE

2,034,643

## MOTOR FUEL

René de M. Taveau, Newburgh, N. Y., assignor to  
The Texas Company, New York, N. Y., a corporation of Delaware

No Drawing. Application June 1, 1933,  
Serial No. 673,853

10 Claims. (Cl. 44—9)

This invention relates to improvements in motor fuels for internal combustion engines of the Diesel or compression ignition type, and is particularly concerned with the provision of a combustion primer or accelerator in the fuel for the purpose of inducing ignition at lower compression pressures or compression ratios than would be possible without such an accelerator. 5

Time lag is a phenomenon which is prevalent in practically all types of compression ignition engines and is defined as the length of time occurring between the entrance of the first portion of the fuel charge into the engine cylinder and its subsequent ignition. Time lag is principally responsible for undesirable engine operation characteristics known as detonation, misfiring, and rough running, and the longer the time lag the worse these conditions become. However, time lag with its accompanying evils can be reduced ordinarily by either increasing the compression ratio of the engine, or by changing the characteristics of the fuel itself in such a way as to reduce the compression ratio necessary for ignition. Obviously the first remedy, that of increasing the compression ratio, is not mechanically possible in many engines and is undesirable in all since the structural strength and weight of the engine must be considerably increased in order to safely withstand the resulting higher pressures. Such a change also tends to reduce the overall brake thermal efficiency of the engine. The second remedy, that of reducing the minimum compression ratio necessary for the autoignition of the fuel, is therefore the only remedy in many instances and the best in all instances. 35

It is the chief object of the present invention to produce a novel fuel which will meet the compression ignition requirements for various Diesel engines and to provide a simple and efficient method of treating fuels to form products having the desirable compression ignition properties from any oil or from various oils requiring widely different compression ratios for autoignition.

In accordance with the present invention I add to a high boiling or relatively non-volatile fuel, such as commonly used for compression ignition engines, an accelerator comprising a volatile polysulfide, such as an organic tetrasulfide. I may use symmetrical tetrasulfides of the general formula  $R-S-S-S-S-R$  where R may be an alkyl or aryl substituent, or an unsymmetrical compound of the general formula  $R-S-S-S-S-R'$  in which R and R' are unlike constituents, say, R an alkyl or substituted alkyl, and R' an aryl or substituted aryl group. The alkyl substituents

contemplated may be methyl, ethyl, propyl, butyl and other radicals of the higher homologues of the paraffin series, or the corresponding unsaturated radicals of the homologues of the ethylene series. The aryl substituents include phenyl, tolyl, xylyl and other homologues of the benzene series. It is to be understood that I may use substituted alkyl or aryl groups, such as aralkyl and alkyl or aryl radicals containing halogen, amino, hydroxy or methoxy substituents. Compounds which are useful include, for example, diethyl-, diphenyl-, ditolyl-, ethyltolyl, dinitrodiethyl-, and dianisol-tetrasulfides.

The tetrasulfides may be prepared according to methods described in the literature to which reference is made, particularly Annalen, 359, 81 (1907) and J. F. prokt. Chem., (2) 37, 207-13, (1888).

The quantity of the accelerator required for the purpose of reducing the compression ratio for autoignition of the fuel oil in compression ignition engines is usually small; for example, 0.5 to 5.0% and preferably in the region of 1% by weight of the fuel oil.

The compression ratio for autoignition varies with the fuel and is a property inherent in the nature of the ingredients of which the fuel is composed; for example, iso-octane, although lighter than oils ordinarily found in Diesel fuels, performs well in spark-fired engines, but it is a poor fuel for compression ignition engines. On the other hand, n-heptane has good ignition properties for a Diesel fuel but it is a poor fuel for spark-fired engines. In comparing Diesel oils, blends of iso-octane and n-heptane are often made use of as reference fuels, whereby high octane numbers, which indicate useful high compression ratios and characterize the desirable qualities in fuels for spark-fired engines, are usually indicative of undesirable qualities in compression ignition engines; and conversely, high heptane numbers characterize good Diesel fuels or those ignitable at low compression ratios but indicate that the fuels are poor for spark ignition engines. In the examples that are to follow, heptane numbers, i. e., the percentage of heptane in a blend of n-heptane and iso-octane which will give the same minimum compression ratio as that required to effect autoignition of the unknown fuel, will be used as a measure of desirable ignition qualities instead of actual compression ratios.

The following examples will illustrate the operation of the invention.

To a gas oil from an asphaltic base crude oil and having a heptane value of 64 was added ap-

proximately 1% by weight of diethyl-tetrasulfide. The heptane value of the resulting product was 85, or an increase of 21.

To another sample of the same oil was added 5 about the same amount of di-p-tolyl-tetrasulfide and the heptane value of the mixture was 76, or an increase in heptane value of 12.

The above heptane values were determined on 10 a cooperative fuel research variable compression engine adapted to use a standard Bosch solid injection fuel system.

Obviously many modifications and variations of 15 the invention, as hereinbefore set forth, may be made without departing from the spirit and scope thereof, and therefore only such limitations should be imposed as are indicated in the appended claims.

I claim:

- 20 1. The method of accelerating ignition of liquid fuels for internal combustion engines of the Diesel type wherein ignition of the fuel is effected by compression of air in the engine cylinder, which comprises incorporating into the fuel prior to ignition in the engine, in sufficient amount to substantially reduce the compression ratio for auto-ignition, a compound of the general formula R—S—S—S—R in which R is a hydrocarbon radical.
- 25 2. The method of accelerating ignition of liquid fuels for internal combustion engines of the Diesel type wherein ignition of the fuel is effected by compression of air in the engine cylinder, which comprises incorporating into the fuel prior to ignition in the engine, in sufficient amount to substantially reduce the compression ratio for auto-ignition, a compound of the general formula R—S—S—S—R in which R is a hydrocarbon radical.
- 30 3. The method of accelerating ignition of liquid fuels for internal combustion engines of the Diesel type wherein ignition of the fuel is effected by compression of air in the cylinder, which comprises providing in the fuel-air mixture prior to

ignition in the engine, in sufficient amount to substantially reduce the compression ratio for auto-ignition, a compound of the general formula R—S—S—S—R' in which R is an alkyl radical and R' an aryl radical.

4. The method of accelerating ignition of liquid fuels for internal combustion engines of the Diesel type wherein ignition of the fuel is effected by compression of air in the engine cylinder, which comprises incorporating in the fuel prior to ignition a small amount of di-p-tolyl-tetrasulfide compound.

5. The method of accelerating ignition of liquid fuels for internal combustion engines of the Diesel type wherein the ignition of the fuel is effected by compression of air in the cylinder, which comprises providing in the fuel-air mixture prior to ignition in the engine ethyltolyl-tetrasulfide in sufficient amount to reduce the compression ratio for auto ignition.

6. A fuel oil of the class of Diesel oils, for use in compression ignition engines, and containing in sufficient amount to reduce the compression ratio for auto ignition an ignition accelerating compound of the general formula R—S—S—S—R in which R is a hydrocarbon radical.

7. A fuel oil according to claim 6 in which the ignition accelerating compound is diethyl-tetrasulfide.

8. A fuel oil according to claim 6 in which the ignition accelerating compound is di-p-tolyl-tetrasulfide.

9. A Diesel fuel of the class of high boiling hydrocarbon oils, and containing a small amount of an ignition accelerating compound having the general formula R—S—S—S—R', in which R is an alkyl radical and R' an aryl radical.

10. A fuel according to claim 9 in which the accelerating compound is ethyltolyl-tetrasulfide.

RENE DE M. TAVEAU.

5

10

20

25

30

35

40